

Jan. 2, 1934.

R. M. BOEHM

1,941,536

HARD VEGETABLE FIBER PRODUCT OF HIGH STRENGTH AND PROCESS OF MAKING SAME

Filed May 18, 1932



INVENTOR  
*Robert M. Boehm,*  
BY  
*Dyke and Schaines,*  
ATTORNEYS

## UNITED STATES PATENT OFFICE

1,941,536

HARD VEGETABLE FIBER PRODUCT OF  
HIGH STRENGTH AND PROCESS OF MAK-  
ING SAMERobert M. Boehm, Laurel, Miss., assignor to  
Masonite Corporation, Laurel, Miss., a corpo-  
ration of Delaware

Application May 18, 1932. Serial No. 612,072

9 Claims. (Cl. 154—2)

My invention relates to hard, hot-pressed products, as for example boards, of vegetable fiber, and more particularly to such a board or other product having increased strength as measured, for example, by modulus of rupture. For convenience, I will refer to such products as board.

The objects of the invention include among others, the provision of a hard board or other product, of vegetable fiber, that has high strength, and at the same time is free from surface defects known as water spots, and the securing of high strength and high values of other valuable properties, such as water resistance, wet 10 strength, resistance to abrasion and the like in a hot-pressed vegetable fiber board by relatively short time treatment, and without resort to pressures productive of undesirably high density. Other objects will appear from the following de- 15 scription.

Vegetable fiber material for use with my invention may be obtained from various sources, such as hard woods, soft woods, wood forming grasses such as bamboo, cane, straw, or other 20 fibrous vegetable material.

The preparation of the fiber can be accomplished in various ways in which the non-cellulose constituents are largely retained, as for example, by explosion or by grinding, or in other mechanical fashion, or by semi-chemical cooks, or partly by such cooks and partly mechanically, etc.

A raw fiber such as mechanically prepared or exploded fiber, or partially raw fiber such as semi-chemical fiber is preferred, not only on account 35 of greater yield of board and relatively lower cost, but because of self-bounding properties due to retention of non-cellulose, high resistance to absorption of water and high wet strength, all of which are present to the greatest extent in 40 the board made of the raw ligno-cellulose fiber, and to a considerable extent when the raw fiber is produced by semi-chemical cooks or by the combination thereof with mechanical treatment, etc.

The fiber is preferably refined as in a Claffin, or rod-mill, or other refiner, to a sufficient extent to be readily formed into a smooth blanket or wet-lap in a Fourdrinier or equivalent machine, and after such formation, preferably followed by

50 passing through between press rolls, is made into a hard board by simultaneous application of heat and pressure, followed up as shrinkage occurs and maintained until the board is dry. In the case of making a board of about 1 specific 55 gravity, and about one-eighth inch thick, at say

300° F. and a pressure of say 200 pounds per square inch, this requires about fifteen to twenty minutes.

A wire mesh screen is preferably interposed between one face of the board and a press platen 60 to permit ready escape of moisture. The other surface is desirably a smoothly polished surface made, for example, against a smooth surface plate of chromium plated steel.

With raw ligno-cellulose fiber sufficiently refined to make a smooth wet-lap and introduced into the hot press when containing say 60% of water, if the pressure applied is sufficient to give a board of such strength as to show a modulus of rupture as high as above 6,000, surface defects 65 are likely to appear, especially on the smooth polished surface, that are known as water spots, and furthermore, the density will ordinarily exceed a specific gravity of 1, whereas, if the pressure be kept lower when it is desired to make 70 a board of lower density, then, while the board will be free from water spot defects, it will be relatively lacking in strength.

By my invention, I obtain a board of strength materially over modulus of rupture 6,000, without 75 resort to pressures sufficient to produce water spotting or give a high density, as for example, I can secure such high strength in a board made under pressures giving a density considerably under specific gravity 1, which low density board 80 is desirable for purposes where excessive weight and undue thinness are not wanted.

In carrying out my new process, I include or incorporate material adapted to impart high strength to the board or other product when same 85 is subjected to a baking operation in presence of atmospheric or other oxygen, and I subject the board to such baking operation preferably by means of heated air and with provision for efficient air circulation. Materials having drying 90 characteristics can be used in this way such as tung oil, linseed oil, and perilla oil, or mixtures thereof, or less preferably, materials such as rape oil, cottonseed oil, and the like may be used, preferably in admixture with the more desirable materials above referred to, or with admixture of suitable drying accelerators, and other materials operating in substantially the same way can be used.

I purposely avoid inclusion or incorporation of 105 such materials or mixtures to such an extent as to produce saturation of the board, which, with a board of say 1 specific gravity, would require about 15% to 20% of the strength imparting material, as tung oil for example.

- This is not merely because of the economy so obtained in cost of materials, but because of the desirability of performing the baking operation so as to secure the highest strengthening effect 5 in the shortest practicable time, and therefore at the highest practicable temperatures. I find that if the drying oil or other strength imparting agent is present or incorporated to an extent at all approaching saturation, even though the surface 10 excess thereof be wiped or otherwise removed from the surface of the board, when the board containing so much of the drying agent or the like is subjected to substantially high temperature for rapid baking, e. g. 300° F., an effect is 15 quickly produced, which is apparently of a sealing character and productive of lack of access of atmospheric oxygen to the inner portion of the board. The result is that further baking, for any period that is commercially acceptable as say 6 20 hours or under, does not materially increase strength, and the strength may even be reduced instead of increased, this being apparently due to a softening action of the considerable percentage of tung oil or other material present in the board. 25 By using a relatively small proportion of the material having drying characteristics, such as tung oil, for example, say 4% thereof, of the dry weight of fiber, I avoid producing such an oxygen excluding effect as just described, and perform the baking 30 rapidly and efficiently and get good increase in strength in a short time without undue necessity of holding the baking temperature down.
- The material having drying characteristics can be substantially uniformly distributed throughout 35 the entire thickness of the board or other product, by introduction thereof into the pulp from which the fiber mass is formed. Such a board or other product is preferably waterproofed by incorporating a waterproofing agent such as rosin or a 40 hydrocarbon material in the pulp. About 1½% of hydrocarbon material, such as petrolatum, is an effective waterproofing agent, and when the material that is used having drying characteristics is tung oil, for example, the petrolatum or other 45 waterproofing material may be conveniently dissolved in the tung oil and the mixture incorporated with the fiber in the mixing chest before being de-watered and formed into the fiber mass or wet-lap from which the board is made by hot pressing, or the material with drying characteristics 50 may be applied otherwise, as for example applied to the wet-lap after same is formed.
- If it is desired to incorporate the entire content of strengthening agent, as tung oil, in any of 55 the foregoing ways, same may advantageously be about say 4% of the weight of dry fiber. It appears to be substantially entirely taken up by the fiber with little or no loss thereof during the de-watering and hot pressing operations.
- 60 An alternative way of introducing all or part of the strengthening material used is by impregnation treatment of the hard board, after same has been formed by hot pressing. This treatment may consist, for example of dipping or submerging the hard board in a bath of strengthening agent such as tung oil, followed by passing it through between high pressure rollers, which may be disposed below the surface of the bath if desired. Such roller treatment compresses the 65 board progressively along a narrow transverse region and absorption of the treating material is believed to take place as the result of suction effect obtained by the expansion of the board after being subjected to such compression.
- 70 When the boards are smooth and polished on 75 one face and contain a wire mesh impression surface on the other face, the latter face will take up somewhat more of the treating material than the smooth polished face, if both be subjected to the same treatment. To avoid uneven distribution, I preferably make a preliminary application of the treating material to the smooth polished face only, whereby same is taken up to some extent in that side alone, and when later the tung oil or other material is applied alike to the two sides of the board as by submerging in the bath, even penetration will finally be obtained on both faces, and any warping of the board which might result from unequal penetration of the tung oil or other material can be minimized or avoided. 80
- I find that when using tung oil, it is desirable to incorporate about 5% of cottonseed oil therewith (i. e. 5% of the oil bath) in order to avoid a tendency of the tung oil to thicken up, particularly after being subjected to fairly high heating over a considerable period, as heating to around 150° F., which is desirable in order to secure good penetration of the board. If desired, a thinning and penetration-aiding material such as a light 85 paraffin hydrocarbon may be incorporated in the bath, and may form up to about 50% of the treatment bath. 90
- The first described mode of including the strength giving agent in the fiber mixing chest 95 is of advantage in securing uniform distribution throughout the thickness of the fiber mass and resulting board. The impregnation mode just described has the advantage that the inclusion of tung oil or other strength giving material is greatest at the surfaces and the resulting improvement upon baking in properties such as strength and hardness is likewise greatest at the surfaces, which are of course, exposed in use and should desirably have the best properties. 100
- 110 However, I have found that a combination of the two modes for inclusion of the strength giving material to be preferable, namely, by securing uniform distribution throughout the board or other body of one portion, preferably about one-half of the strength-giving agent used, through preliminary incorporation thereof in the fiber, and incorporating the other portion, preferably approximately the remaining one-half, of the strength giving agent by the impregnation route. 115
- In this way, the central zone of the board will contain the strength giving material to some extent through the introduction of a part thereof into the fiber in which it was substantially uniformly distributed, and the parts adjacent to the 120 surfaces, while containing same to an additional extent, do not carry all thereof, as may happen with impregnation alone. 125
- To obtain increased strength by the inclusion or incorporation of material having drying characteristics, the board is baked in presence of oxygen as for example with free access of air, and the temperature may be adapted to the particular drying oil material used, as for example, when using tung oil, about 300° F. With this temperature and using about 5% of tung oil in a hard board of raw ligno-cellulose fiber of specific gravity about 1, the baking will be completed in about six hours, at which time without material density increase, the strength increase is notable and the modulus of rupture is frequently nearly doubled. 130 With tung oil, the final hardening that is complete at the end of the baking period, is believed to be preceded by an intermediate polymerization 135 which transforms the tung oil into substan- 140
- 145

tially a spongy state favorable to getting thorough access of air and hence oxygen. It is desirable to provide for good air circulation during baking, and for this reason baking by means of 5 heated air is preferred.

The impregnation and baking treatments may be repeated one or more times if desired and similar advantage obtained though generally to a relatively lesser degree.

10 After the baking is completed, the board is preferably humidified to equalize its moisture content with atmospheric moisture and is ready for use.

The accompanying drawing comprises a series 15 of curves showing actual instances of baking time, at a temperature of 300° F., plotted against modulus of rupture for boards of raw ligno-cellulose fiber of 1.02 specific gravity for 5%, 10% and 15% content of tung oil, and it will be noted 20 that in 6 hours baking time the board with the 5% of tung oil (top curve) had its modulus of rupture increased from 6150 to substantially the maximum for any time period, namely 10,500, an increase of 73%; whereas for 10% tung oil 25 (middle curve) the increase in strength in 6 hours was from 6150 to 7600 or 23%, and further increase was obtained only at the expense of very prolonged baking; and for 15% tung oil (lowermost curve), instead of an increase of strength 30 as represented by modulus of rupture there was a decrease in 6 hours from 6150 to 5900, or a decrease of 4%.

In addition to securing a very desirable increase in the strength and related properties of 35 the board at substantially minimum expense for material and treatment, with absence of troubles from surface defects, such as water spots and the like, and without the necessity of producing a board of extremely high specific gravity, I also 40 obtain further advantages by my invention as for example, an increase in tensile strength is obtained to approximately the same extent as that in modulus of rupture, and similar benefits obtained in resistance to absorption of water, in 45 wet strength and in fire resistance; the modulus of elasticity is materially increased, and there is a tremendous increase, amounting to practically five-fold, in resistance to abrasion. Also the appearance of the product is enhanced, less

coats of paint, varnish, enamel or other finish material are required for getting a good finish surface, and yet other features of advantage obtained.

I claim:

1. The process of making a fiber product of great dry and wet strength which comprises subjecting to consolidating pressure and heat until dry a moist mass of vegetable fiber having a sufficiently large non-cellulose content to bond the fibers together, and in subjecting the same with a drying oil content the quantity of which is less than one-half that which is necessary to saturate the mass after consolidation, to highly heated air for a sufficient time to greatly increase the modulus of rupture of the material. 80
2. The process of claim 1 in which the drying oil is tung oil, the heated air is at a temperature of about 300° F., and the time during which the material is subjected to heated air is less than 85 seven hours. 90
3. The process of claim 1 in which the drying oil is tung oil to the extent of approximately 4% of the weight of dry fiber. 95
4. The process of claim 1 in which the drying oil is incorporated into the vegetable fiber mass before it is consolidated by heat and pressure. 100
5. The process of claim 1 in which the drying oil is incorporated into the vegetable fiber material after it has been consolidated by heat and pressure. 105
6. The process of claim 1 in which some of the drying oil is incorporated into the vegetable fiber mass before and some after it is consolidated by heat and pressure. 110
7. A hard vegetable fiber product such as board and the like having great dry and wet strength and composed of compressed vegetable fiber bonded together by non-cellulose and a hardened drying oil material in quantity less than one-half that which is necessary to saturate the compressed fibrous material. 115
8. The product of claim 7 in which the drying oil includes tung oil. 120
9. The product of claim 7 in which the drying oil is tung oil in quantity of approximately 4% of the weight of the dry fiber. 125

ROBERT M. BOEHM.

Patent No. 1,941,536.

January 2, 1934.

ROBERT M. BOEHM.

It is hereby certified that error appears in the printed specification of the above numbered patent requiring correction as follows: Page 1, line 36, for "self-bounding" read self-bonding; and that the said Letters Patent should be read with this correction therein that the same may conform to the record of the case in the Patent Office.

Signed and sealed this 27th day of February, A. D. 1934.

F. M. Hopkins

Acting Commissioner of Patents.

(Seal)

tially a spongy state favorable to getting thorough access of air and hence oxygen. It is desirable to provide for good air circulation during baking, and for this reason baking by means of 5 heated air is preferred.

The impregnation and baking treatments may be repeated one or more times if desired and similar advantage obtained though generally to a relatively lesser degree.

10 After the baking is completed, the board is preferably humidified to equalize its moisture content with atmospheric moisture and is ready for use.

The accompanying drawing comprises a series 15 of curves showing actual instances of baking time, at a temperature of 300° F., plotted against modulus of rupture for boards of raw ligno-cellulose fiber of 1.02 specific gravity for 5%, 10% and 15% content of tung oil, and it will be noted 20 that in 6 hours baking time the board with the 5% of tung oil (top curve) had its modulus of rupture increased from 6150 to substantially the maximum for any time period, namely 10,500, an increase of 73%; whereas for 10% tung oil 25 (middle curve) the increase in strength in 6 hours was from 6150 to 7600 or 23%, and further increase was obtained only at the expense of very prolonged baking; and for 15% tung oil (lowermost curve), instead of an increase of strength 30 as represented by modulus of rupture there was a decrease in 6 hours from 6150 to 5900, or a decrease of 4%.

In addition to securing a very desirable increase in the strength and related properties of 35 the board at substantially minimum expense for material and treatment, with absence of troubles from surface defects, such as water spots and the like, and without the necessity of producing a board of extremely high specific gravity, I also 40 obtain further advantages by my invention as for example, an increase in tensile strength is obtained to approximately the same extent as that in modulus of rupture, and similar benefits obtained in resistance to absorption of water, in 45 wet strength and in fire resistance; the modulus of elasticity is materially increased, and there is a tremendous increase, amounting to practically five-fold, in resistance to abrasion. Also the appearance of the product is enhanced, less

coats of paint, varnish, enamel or other finish material are required for getting a good finish surface, and yet other features of advantage obtained.

I claim:

1. The process of making a fiber product of great dry and wet strength which comprises subjecting to consolidating pressure and heat until dry a moist mass of vegetable fiber having a sufficiently large non-cellulose content to bond the fibers together, and in subjecting the same with a drying oil content the quantity of which is less than one-half that which is necessary to saturate the mass after consolidation, to highly heated air for a sufficient time to greatly increase the modulus of rupture of the material. 80
2. The process of claim 1 in which the drying oil is tung oil, the heated air is at a temperature of about 300° F., and the time during which the material is subjected to heated air is less than 85 seven hours. 90
3. The process of claim 1 in which the drying oil is tung oil to the extent of approximately 4% of the weight of dry fiber. 95
4. The process of claim 1 in which the drying oil is incorporated into the vegetable fiber mass before it is consolidated by heat and pressure. 100
5. The process of claim 1 in which the drying oil is incorporated into the vegetable fiber material after it has been consolidated by heat and pressure. 105
6. The process of claim 1 in which some of the drying oil is incorporated into the vegetable fiber mass before and some after it is consolidated by heat and pressure. 110
7. A hard vegetable fiber product such as board and the like having great dry and wet strength and composed of compressed vegetable fiber bonded together by non-cellulose and a hardened drying oil material in quantity less than one-half that which is necessary to saturate the compressed fibrous material. 115
8. The product of claim 7 in which the drying oil includes tung oil. 120
9. The product of claim 7 in which the drying oil is tung oil in quantity of approximately 4% of the weight of the dry fiber. 125

ROBERT M. BOEHM.

Patent No. 1,941,536.

January 2, 1934.

ROBERT M. BOEHM.

It is hereby certified that error appears in the printed specification of the above numbered patent requiring correction as follows: Page 1, line 36, for "self-bounding" read self-bonding; and that the said Letters Patent should be read with this correction therein that the same may conform to the record of the case in the Patent Office.

Signed and sealed this 27th day of February, A. D. 1934.

F. M. Hopkins

Acting Commissioner of Patents.

(Seal)